

1

3,376,174

**POWDER CONTAINING NITROCELLULOSE,  
METAL OR METAL HYDRIDE AND A  
SUPERFICIAL LAYER OF MODERATING  
AGENT**

Claude Napolé, Finistère, Jean-Jacques Humbert, Charente, and Alain Lamboley, Puteaux, France, assignors to Etat Français, représenté par le Ministre, des Armées, Délégation Ministérielle pour l'Armement, Paris, France  
No Drawing. Filed Sept. 16, 1966, Ser. No. 579,820  
Claims priority, application France, Sept. 21, 1965,

32,029

4 Claims. (Cl. 149—13)

2

sufficiently regular and progressive combustion in order to impart the maximum impulse to the projectile.

The present invention has the object of providing a granular powder for mortar shell cartridges having the following characteristics:

Satisfactory ignition irrespective of the filling coefficient, the position of the powder charge in the case, and the initial temperature;

Higher resistance to extinction even under highly adverse conditions and with low initial temperatures;

Steadiness of the manner in which the major part of the powder burns after opening of the cartridge and projection of the powder charge into the tube.

For this purpose the granular powder according to the invention is composed of a major part of nitrocellulose or an organic nitrate or a mixture of nitrocellulose and an organic nitrate and also contains:

(a) On the one hand, in a manner uniformly distributed throughout the mass, a metal or a metallic compound which is finely divided and is a good conductor of heat having a high energy of combustion and which ignites only in the gases at a temperature above a predetermined level which is a function of the nature of these gases, such as aluminium, magnesium, beryllium, lithium, lithium hydride or the like;

(b) On the other hand in a superficial layer in addition to the metal or metallic compound, a moderating agent which can be introduced by a glossing technique, such as centralites, particularly ethyl centralite, 2,4-dinitrotoluene and 2,6-dinitrotoluene, camphor, diphenylamine, urethanes and similar materials.

The thermal conductivity of the metals used is always much greater than that of the powders. As regards their energy of combustion, this can be characterised by the apparent potential of the metal which should be higher than that of the powder, the metals or metallic compound chosen having an apparent potential greater than 2000 cal./g.

The amount of metal or metallic compound can range from 0.5% to 10% according to the nature of the metal or metallic compound and the operating characteristics of the shell. However it should be sufficiently high for the powder to have sufficient properties of ignition and a resistance to extinction without being high enough for the combustion products to cause too large an erosive action on the mortar as a result of a high combustion temperature and the presence of solid compounds in the combustion products of the powder.

The amount of the moderator can range from 0.5—20% according to the nature of the moderator and that of the metal or metallic compound introduced into the powder. It should always be sufficiently high for the combustion temperature of the superficial layer of the powder to be lower than the combustion threshold of the metal or the metallic compound contained in the powder. Also it should be sufficiently low for the combustion temperature under constant volume of the superficial layer of the powder to be greater than 1800° K., the ignition of the powders below this value being very difficult to achieve.

60 The incorporation in the proposed propulsive powders of metals or metallic compounds of this type allows the powders to burn in a stable manner at a lower pressure than for propulsive powders not containing them.

These metals and metallic compounds incorporated in the propulsive powders in a finely divided form burn in the combustion gases of the propulsive powders when their temperature is sufficiently high (the minimum limiting temperature in the case of aluminium being about 2300° K.) and thus increase significantly the energy evolved by the powder.

Also the moderators have the ability to be fixed in an external layer of greater or lesser thickness formed from

**ABSTRACT OF THE DISCLOSURE**

The present invention is directed to propulsive powders for mortar shells. The powder comprises a granular mixture of a major proportion of a propulsive organic nitrate preferably nitrocellulose and a powdered metal or metal compound such as aluminum, magnesium, beryllium, lithium and lithium hydride. The granular powder mixture in addition possesses a superficial layer of a moderator such as centralites, dinitrotoluene, camphor, diphenylamine and urethanes which is applied by a glossing technique. Preferred powders contain from 0.5 to 10% by weight of the metal or metallic compound and from about 0.5% to 20% by weight of the moderator.

The firing of mortar shells is effected by ball-less cartridges, containing a propulsion powder charge enclosed in a case which is sealed by a mount folded in upon a sealing varnish. The pressure of the combustion gases acts upon the base of the mortar shell, the stem of which, pushed into the end of the tube, acts as a piston. Although the principle as such is thus very simple, it has always been extremely difficult to make this system function in a convenient and reproducible manner.

The absence of a projectile set upon the case of the cartridge and limiting the expansion of the combustion gases in the mortar causes the creation of an undulatory pressure system which is responsible for the large variations in the values of the maximum pressures. Experimental measurements have shown that the wave has time to travel, out and back, two or three times the length of the tube before the mortar shell is expelled and no longer serves as a reflector. The amplitude of the wave diminishes rapidly with reflections, but during the first transit it is so high that it often involves rupture of the feathering of the mortar.

Also the powder is ignited inside the sealed cartridge. As the filling coefficient (i.e. the ratio of the useful charge to the charge occupying the interior volume of the cartridge), of all kinds of mortar shell cartridges filled with known powders is not sufficient, ignition occurs under adverse conditions which is the cause of considerable variations of velocity and pressure. Moreover under the pressure of the gases produced by the powder on combustion, the forward end of the cartridge opens and the compressed gases escape into the tube. The sudden decompression which results inside the cartridge causes partial extinction to a greater or lesser extent of the powder when it is insufficiently ignited or when it has too low a resistance to extinction.

In order to remedy the extinction of a significant part of the powder, it has been proposed in French patent specification No. 1,311,647 to add to the powder a strongly exothermic reactant, such as paraphenylenediamine. But this additive alone, although it facilitates combustion of the powder does not provide for the propulsive unit a



(b) as a superficial layer in addition to the metal or metallic compound, from about 0.5% to about 20% by weight of a moderating agent having an imaginary negative apparent potential or low positive apparent potential, said moderating agent being capable of being introduced by a glossing technique and selected from the group consisting of centralites, dinitrotoluenes, camphor, diphenylamine and urethanes, said moderating agent being present in such quantity that the gases produced upon ignition of said powder by the layer containing the moderator have a temperature between the temperature at which there is no stable burning and the temperature above which detonation of the incorporated metal would be produced.

2. A powder according to claim 1 having the following percentage composition by weight:

|                                         | Percent |
|-----------------------------------------|---------|
| Nitrocellulose (nitrogen content 13.2%) | 92.5    |
| Aluminium powder                        | 5.0     |
| Diphenylamine                           | 1.5     |
| Potassium cryolite                      | 1.0     |

and 2% by weight of a moderator selected from the group

consisting of centralites, dinitrotoluenes, camphor diphenylamine and urethanes which is introduced into the external layer by a glossing technique.

3. A powder according to claim 2 wherein the moderator is ethyl centralite.

4. A powder according to claim 1 wherein the metal is aluminum.

#### References Cited

##### UNITED STATES PATENTS

|           |         |                 |       |          |
|-----------|---------|-----------------|-------|----------|
| 3,118,797 | 1/1964  | Coffee          | ----- | 149—38 X |
| 3,222,233 | 12/1965 | Matuszko et al. | ----- | 149—38   |
| 3,236,704 | 2/1966  | Axelrod et al.  | ----- | 149—99 X |

##### OTHER REFERENCES

Federoff et al., Encyclopedia of Explosives and Related Items, vol. 2, Picatinny Arsenal, Dover, N.J., 1962, pp. C 126 to 140.

CARL D. QUARFORTH, Primary Examiner.

LELAND A. SEBASTIAN, Examiner.